# EUROPEAN PATENT SPECIFICATION

(11) **EP 1 691 005 B1**
(45) Date of publication and mention of the grant of the patent: **19.08.2009**
(21) Application number: 05003173.1
(22) Date of filing: 15.02.2005
(51) Int. Cl.: E04F 15/04, B44C 5/04, B27M 3/04

(54) **Method to make a floorboard with compressed edges**
Methode zur Herstellung von Fussbodenplatten mit komprimierten Kanten
Procédé de fabrication de planches der plancher avec des bords comprimés

(43) Date of publication of application: 16.08.2006
(73) Proprietor: Välinge Innovation AB, 260 40 Viken (SE)
(72) Inventor: Pervan, Darko, 260 40 Viken (SE)
(74) Representative: Åkesson, Sten Jan-Åke

(56) References cited:
- DE-U1- 20 317 527
- FR-A- 2 846 023
- JP-A- 2003 200 405
- US-A- 1 790 178
- US-A- 4 084 996
- US-A- 4 612 074
- PATENT ABSTRACTS OF JAPAN vol. 2000, no. 24, 11 May 2001 (2001-05-11) & JP 2001 179710 A (DAIKEN TRADE & IND CO LTD), 3 July 2001 (2001-07-03)
- PATENT ABSTRACTS OF JAPAN vol. 2000, no. 26, 1 July 2002 (2002-07-01) & JP 2001 260107 A (UCHIYAMA MFG CORP), 25 September 2001 (2001-09-25)
- PATENT ABSTRACTS OF JAPAN vol. 2000, no. 26, 1 July 2002 (2002-07-01) & JP 2001 254503 A (TOYO TEX CO LTD), 21 September 2001 (2001-09-21)
- PATENT ABSTRACTS OF JAPAN vol. 007, no. 031 (M-192), 8 February 1983 (1983-02-08) & JP 57 185110 A (AIKA KOGYO KK), 15 November 1982 (1982-11-15)

## Description

### Technical field

The present invention generally relates to floorboards, which have a wood fiber based core, a surface layer and compressed curved edge portions. More particularly, the present invention relates to interlocked floorboards with compressed edge portions located below the panel surface. The invention relates to panels with such edge portions and to a method to produce such panels.

### Field of Application of the Invention

The present invention is particularly suitable for use in floating floors, which are formed of floorboards comprising a wood fiber based core with a surface layer and which are preferably joined mechanically with a locking system integrated with the floorboard. A floorboard with a mechanical locking system has a rather advanced edge profile and curved edge portion are more difficult produce than in traditional furniture components. The following description of prior-art technique, problems of known systems and objects and features of the invention will therefore, as a non-restrictive example, be aimed above all at this field and in particular to laminate flooring with mechanical locking systems. However, it should be emphasized that the invention can be used in optional floorboards with optional locking systems, where the floorboards have a core and at least one surface layer and where these two parts are possible to be formed with a pressure force applied to the surface layer. The invention can thus also be applicable to, for instance, floors with one or more surface layers of wood applied on a wood fiber core. The present invention could also be used in building panels i.e. wall panels, ceilings and floor strips such as dilatation profiles, transition profiles or finishing profiles.

### Definition of Some Terms

In the following text, the visible surface of the installed floorboard is called **"front side",** while the opposite side is called **"rear side". "Horizontal plane"** relates to a plane, which extends along the outer flat parts of the surface layer at the front side. **"Vertical plane"** relates to a plane, which is perpendicular to the horizontal plane and at an outer edge of the surface layer. By **"up"** is meant towards front side, by **"down"** towards rear side, by **"vertical"** parallel with the vertical plane and by **"horizontal"** parallel with the horizontal plane.

By **"edge portion"** is meant a part of the edge, which is below the horizontal plane. **By "floor surface"** is meant the outer flat parts of the surface layer along the horizontal plane. By **"edge surface"** is meant the surface of the edge portion. By **"locking system"** is meant cooperating connecting means, which interconnect the floorboards vertically and/or horizontally. By **"mechanical locking system"** is meant that joining can take place without glue.

### Background of the Invention, Prior-Art Technique and Problems thereof.

Laminate floors and other similar floorboards are made up of one or more upper layers of decorative laminate, decorative plastic material or wood veneer, an intermediate core of wood fiber based material or plastic material and preferably a lower balancing layer on the rear side of the core.

Laminate flooring usually consists of a core of a 6-9 mm fiberboard, a 0.2-0.8 mm thick upper decorative surface layer of laminate and a 0.1-0.6 mm thick lower balancing layer of laminate, plastic, paper or like material. The surface layer provides appearance and durability to the floorboards. The core provides stability, and the balancing layer keeps the board plane when the relative humidity (RH) varies during the year. The floorboards are laid floating, i.e. without gluing, on an existing subfloor. Traditional hard floorboards in floating flooring of this type are usually joined by means of glued tongue-and-groove joints.

In addition to such traditional floors, floorboards have been developed which do not require the use of glue and instead are joined mechanically by means of so-called mechanical locking systems. These systems comprise locking means, which lock the boards horizontally and vertically. The mechanical locking systems can be formed by machining of the core. Alternatively, parts of the locking system can be formed of a separate material, which is integrated with the floorboard, i.e. joined with the floorboard in connection with the manufacture thereof.

The most common core material is a fiberboard with high density and good stability, usually called HDF - High Density Fiberboard. Sometimes also MDF - Medium Density Fiberboard - is used as core. MDF and HDF contain ground wood fibers, which by means of binding agents are combined into a sheet material.

Laminate flooring and also many other floorings with a surface layer of plastic, wood, veneer, cork and the like are produced in several steps. As shown in figure 1a - 1d the surface layer and the balancing layer is produced in a separate step and are then applied to a core material by for example gluing a previously manufactured decorative layer and balancing layer to a fiberboard. Such a production process is used when a floor panel has a surface of a decorative high pressure laminate (HPL) which is made in a separate operation where a plurality of sheets of paper impregnated with a thermosetting resin, such as melamine and/or phenol are compressed under high pressure and at a high temperature.

The currently most common method when making laminate flooring, however, is the direct pressure laminate (DPL) method which is based on a more modern principle where both manufacture of the decorative laminate layer and the fastening to the fiberboard take place in one and the same manufacturing step. One or more papers impregnated with a thermosetting resin such as melamine are applied directly to the board and pressed together under pressure and heat without any gluing.

One prior art method is disclosed in FR 2 846023. To provide an embossing effect, rectilinear lines are pressed into a floor element using an embossing die in the neighbourhood of each intended line of separation. The lines of separation are formed in a later step when cutting out floor panels. In a still later step, locking means are machined in the area between the embossed rectilinear line and the line of separation.

Another prior art method is disclosed in US 4 084 996, wherein the method starts with assembling a number of individual layers such as plywood, wood chips and a fibrous web. The assembly is disposed together with a caul plate in a hot press subjecting it for heat and pressure consolidating and adhering the layers and preserving the surface pattern transferred to the surface by the caul plate. The method is used for producing plywood panels suitable for external uses.

Yet another prior art method is disclosed in JP-A-2003200405. The document discloses a method of providing a facing material for a floor material or the like. An edge part between the upper surface and a side surface is pushed with a hard roll to execute chamfering. The chamfering is made after cutting the panel and after forming coupling means.

Figures 1a - 1d shows how laminate flooring is produced according to known technology. As a rule, the above methods result in a floor element (3 in fig 1b) in the form of a large laminated board, which is then sawn into several individual floor panels (2 in fig 1c), which are then machined to floorboards (1 in fig 1d). The floor panels are individually machined along their edges to floorboards with mechanical locking systems on the edges. The machining of the edges is carried out in advanced milling machines where the floor panel is exactly positioned between one or more chains and belts or similar, so that the floor panel can be moved at high speed and with great accuracy past a number of milling motors, which are provided with diamond cutting tools or metal cutting tools, which machine the edge of the floor panel. By using several milling motors operating at different angles, advanced profiles can be formed at speeds exceeding 100 m/min and with an accuracy of ±0.02 mm.

The upper edges of the floorboards are in most cases very sharp and perpendicular to the floor surface and in the same plane as the floor surface.

Recently laminate floors have been developed with decorative grooves or bevels at the edges, which looks like a real gap or a bevel between solid wood floor such as planks or parquet strips.

It is known that such edges cold be made in several different ways.

In recent years, laminate floors, which are imitations of stones, tiles and the like, have become more and more common. It is known that the method which is used to manufacture decorative edge portions of such floors could also be used to produce edge portions which look like a gap in solid wood floors. This is shown in figure 2a and 2b. The starting material is a decorative paper with printed edge portions which is impregnated with melamine resin. Uncontrolled swelling takes place in this operation. In the subsequent lamination, the decorative impregnated paper is placed on a core and lamination takes place against an embossed metal sheet, which forms a depression (20) in those parts of the floor element (3) where edge portions are to be formed. This is shown in figure 2a. The result is a floor element (1,1') whose front side has an embedded or embossed edge pattern corresponding to the intended edge portions between floorboards, as shown in figure 2b.

This manufacturing method suffers from a number of problems, which are above all related to difficulties in positioning the decorative paper and metal sheets in connection with laminating and the difficulty in positioning floor element and floor panels in the subsequent sawing and machining of the edges. The result is a floor panel with edge portions, which show considerable and undesired variations in structure and design as shown in figure 2b. Another problem is that this method is only suitable for embossed textures which are less than about 0,2 mm deep and which cannot be made deeper than the thickness of the surface layer. Further disadvantages are that although the edge is below the floor surface, it is sharp and parallel with the surface.

Figure 2c and 2d show another method. Decorative edge portions could be made in connection with the machining of the edges of the floor panel 1, 1'. Laminating and sawing of the floor element (3) can then take place without any specific requirements as to alignment, and swelling problems do not occur. The decorative and embedded edge portion can be provided by part of the decorative surface layer being removed so that the reinforcing layer of the laminate becomes visible (figure 2d). Alternatively, the core (30) itself can be used to create the decorative embedded edge portion. This is shown in figure 3a. The surface layer has been removed and the core (30) is uncovered within areas that are to constitute the decorative edge portion (20). A decorative grove could be made on only one edge as shown in figure 3a.

The most common method is shown in figure 3b. A part of the edge portion of a floorboard (1, 1') has been formed as a bevel 20 and this bevel is than in a separate operation covered with a separate material such as a tape, a plastic strip or it could be colored, printed etc. Separate materials are complicated and costly to apply and it is not possible to make an edge portion with the same design and structure as the floor surface. Such edge portion has considerable lower abrasion resistance and inferior moisture properties than the floor surface. The production method is rather slow and several application units are needed to meet the speed of a modern production line for laminate floorings.

Another method is shown in figure 3c. The edge portion (20) is formed in a separate material, which has been inserted or extruded into a groove. This method has the same disadvantages as the method described above.

Fig 3d show that a rounded edge portion (20) could be produced with the well known postforming method used for furniture components. A postforming laminate surface (31) of HPL, which is so flexible that it can be formed after the production of the laminated sheet, could be glued to an already machined floorboard (1). In a second production step the edge could be heated and the laminate could be bent and glued around the edge portion. This method would be very complicated, costly and is not used in laminate floorings.

The principles of the present invention are directed to edge portions in building panels, which overcome one or more of the limitations and disadvantages of the prior art.

These and other objects of the invention are achieved by floorboards, and manufacturing methods having the features that are stated in the independent claims. The dependent claims define particularly preferred embodiments of the invention.

### Summary of the invention

The main objective of this invention is to provide floorboards, with curved edge portions made in one piece with the surface layer, which could be produced more efficiently than present products on the market.

An additional purpose of this invention is to provide such panels with edge portions, which have improved design and abrasion properties.

To achieve these objectives, according to a first principle not forming part of the invention, a floorboard is provided, with locking system, a wood fiber based core and a surface layer arranged on the upper side of the core. The outer flat parts of the surface layer constituting a floor surface and a horizontal plane. A plane, perpendicular to the horizontal plane and at the edge of the surface layer, constitutes a vertical plane. The floorboard has an edge portion with an edge surface, which is located under the horizontal plane. The edge surface at the vertical plane is at a distance from the horizontal plane which constitutes an edge depth and which exceeds the thickness of the surface layer.

The floor surface and the edge surface are made in one piece of the same material. A part of the core in the edge portion under the edge surface adjacent to the vertical plane and at a vertical distance from the edge surface has a higher density than a part of the core under the floor surface adjacent to the edge portion and at the same vertical distance from the floor surface.

According to one principle of the invention, a method is provided to make a floorboard, with a locking system, a wood fiber based core and a surface layer arranged on the upper side of the core. The outer flat parts of the surface layer constituting a floor surface and a horizontal plane. The floorboard has an edge portion with an edge surface, which is located under the horizontal plane. The method comprises the steps of:
- Applying the surface layer on the core to form a floor element.
- Cutting the floor element into floor panels.
- Applying a pressure on the surface of an edge portion of the floor panel such that the core under the surface layer is compressed and the surface layer is permanently bended towards the rear side.

### Brief Description of the Drawings

**Figs 1a****-d** illustrate in different steps manufacture of a floorboard according to known technology.
**Figs 2a****-d** illustrate production methods to form edge portions according to known technology.
**Figs 3a****-d** illustrate examples of different ways of manufacture of edge portions according to prior art.
**Figs 4a****-b** illustrate press forming of a edge portion according to the invention.
**Figs 5a****-c** illustrate different properties of a convex curved edge portion according the invention.
**Figs 6a****-b** Illustrate alternative methods ,the method is not part of the invention.
**Fig. 7** illustrates a dilatation profile according to the which is not considered as being part of the invention.
**Fig. 8** illustrates an edge portion with a curved edge surface.

### Description of Preferred Embodiments

Figs 4a-4c show in four steps manufacture of floorboards according to one embodiment of the invention. Fig. 4a shows two opposite edges of two essentially similar floor panels 2, 2' which are intended to be joined together with a mechanical locking system. The floorboards have a surface layer 31 of for example HPL, DPL or wood veneer, a core 30 of HDF and balancing layer 32. As show in fig. 4b an edge groove 16, 16' is formed at the upper side of the edge and a part of the surface layer 31 is removed. This could be done in a separate operation or in connection with the sawing of the floor element 3 into floor panels 2. If the surface layer 31 is laminate, at least a part of the edge groove 16,16' and the surface layer 31 adjacent to the edge groove 16,16' should preferably be heated with a suitable heating device H, such as for example heating nozzles which blow an even current of hot air. The temperature should exceed 100 degree C. A preferable temperature is about 150 - 200 degree C. In many applications a temperature of about 170 degree C gives the best result. Normal laminate quality could be used as a surface layer 31 and no special post forming quality is needed. If the surface layer 31 is a wood veneer, heating is preferably not required. The floor panel should preferably have a reference surface 17, 17' which could be used to position the floor panel correctly when edge portions and locking systems are formed. As shown in figure 4c the edge portions 20, 20' are than compressed with a compression tool TO which preferably is heated to similar temperatures as described above. The compression tool TO could be a wheel and/or a pressure shoe or similar with a profile which preferably corresponds to the desired edge profile. Several tools could be used to form the edge portion in several steps. During the compression, the fibers in the core will be permanently compressed, the fiber orientations will in most cases change and the density in the edge portion 20 will increase. A change in the fiber orientation might be difficult to detect in some core materials. Increased density could however be measured with grate accuracy. The edge portion 20 will be much stronger than traditional beveled edges in laminate flooring. The abrasion resistance will be similar as in the floor surface and the visible edge portion will have the same design and structure as the floor surface. The upper parts of the core 30 under the surface layer 31, which in a DPL flooring is impregnated with melamine and in a HPL flooring with glue, supports the laminate surface layer 31 during the bending and increases the flexibility of the laminate layer. The advantage is that ordinary qualities of thermosetting decorative laminates, which are rather brittle, could be used. HDF is particularly suitable for this kind of press forming with permanent compression according to the invention since the fiber structure and the binders, which are used in HDF, are ideal for this application.

As shown in figure 4d a mechanical locking system with a tongue 10 and grove 9 for vertical locking and a strip 6 with a locking element 8 and a locking grove 12 for horizontal locking could easily be formed and positioned with high precision in relation to the compressed edge portions 20,20'. In this embodiment the press forming of the edge portions 20, 20' is made on the floor panel 2, which thereafter is machined to a floorboard 1. The advantage is that the forming of the mechanical locking system can be made with great accuracy and the press forming will not change the dimensions of the profile which in this embodiment is mainly the tongue 10 and the groove 9. Of course it is possible to form the edge portions 20, 20' on the floorboard after the machining of the edges, but this is more complicated and the compression possibilities are more limited. In most cases further machining is then required to form the upper outer edge.

Figure 5a shows a cross section of a panel edge according to the invention. In this preferred embodiment the floor panel 1 has a surface layer 31 of DPL with a surface thickness ST and an outer edge 51. The upper flat part of the surface layer 31 constitutes a horizontal plane HP and a floor surface 33. A plane perpendicular to the horizontal plane and at the outer edge 51 of the surface layer 31, constitutes a vertical plane VP. The convex curved edge portion 20, which is located under the horizontal plane HP and which extends to the vertical plane VP has a edge width EW, measured parallel with the horizontal plane HP and an edge surface 50. The edge portion 20 has an edge depth ED measured vertically from the horizontal plane HP, which is equal to the distance SD from the horizontal plane HP to the outer edge 51 at the vertical plane VP. As shown I figure 5a the fibers in the edge portion 20 have been compressed and the fiber orientation have been changed such that the fibers are curved in the same direction as the edge surface 50 of the edge portion 20.

Several relationships are favorable in order to produce an edge portion (20) according to the invention.
- Edge depth ED should preferably be larger than the surface layer thickness ST. In the most preferable embodiment edge depth ED should be larger than 2 or even 3 times the surface thickness ST. The method allows forming of edge portions 20 with edge depths ED exceeding 10 times the surface thickness ST.
- The edge width EW should preferably be larger than the edge depth ED. In the most preferable embodiment edge width EW should be larger than 2 times the edge depth ED
- The edge depth ED should preferably be larger than 0,1 times the floorboard thickness T.
- The thickness ST of the surface layer 31 should be 0,1 - 0,01 times the floor thickness T.

These relationships could be used independently or in combination.

Figure 5b shows the density D profile in a part (A-A) of a floorboard 1 which has not been compressed and figure 5c shows the density profile D in a compressed edge portion (B-B) of the same floorboard. Density profiles could be measured extremely accurately with a gamma beam. The distance between measuring points could be as small as 0,04 mm. In this example the surface layer 31 of laminate, which is about 0,2 mm thick, has a density of about 1300 kg/m3. Below the surface layer 31 there is a core portion 52 which in connection with the direct pressure lamination has been impregnated with melamine and where the density varies between about 1200 - 1000 kg/m3. Under this core portion 52 there is another portion 53 where the density is slightly higher than in the middle parts of the core 30. The average density is shown by the line AD. It should be emphasized that compression in wood fiber based board material always gives an increased density.

Figure 5c shows the density profile in a compressed part B-B of the edge portion 20. A part of the core 30 in the edge portion adjacent to the vertical plane VP and at a vertical distance SD from the surface layer 31, has a higher density D than a part of the core which is under the floor surface adjacent to the edge portion 20 and at the same vertical distance SD from the surface layer 31.

This is contrary to traditional postforming where the edge portion is machined and the surface layer is glued to the part of the core, which have the same or lower density.

Figure 6a shows an alternative method to form an edge portion 20 in a DPL flooring. A floorboard 1 is produced with an edge groove 19 under the surface layer 31. The upper part of the edge grove 19 consist of the surface layer 31 and a part of the core 30. This upper part of the edge grove 19 is folded against the lover part of the edge grove 19 and both parts are pressed and glued together. Figure 6b shows that this method could be used to form an edge portion of a floor panel which is then machined to a floorboard. Both these methods are more complicated than the press forming since glue and separate machining is required. This method could be partly combined with the press forming and the core could be compressed in connection with the gluing.

Figure 7 shows a dilatation profile 4 with press formed edge portions 20, 20', according to the invention.

Figure 8 shows a floorboard with edge portions 20 at opposite edges which are curved and where the outer adjacent parts of the edge surfaces 50 are essential parallel with the horizontal plane HP.

The invention is especially suitable to produce laminate floorings which look like solid wood floor strips with a width of about 5-10 cm and where compressed edge portions are only formed on the long sides. Such floorboards could also easily be made in random lengths since long press formed floor panels could be produced which are thereafter machined and cut to floorboards in different lengths.

A floor which consist of such floorboards will have many curved edge portions 20 and only very cost efficient production methods such as press forming could be used in order to obtain production costs which are competitive and lower than similar solid wood floors.

Press forming is very efficient and can easily meet the speed of modern profiling lines.

The method to compress the core with a surface layer of a laminate floor element, floor panel or floorboard or a similar building element panel according to the invention could be used to form embossed portions on other parts than the edges.

## Claims

1. A method to make a floorboard, with a locking system, a wood fiber based core (30) and a surface layer (31) arranged on the upper side of the core, the outer flat parts of the surface layer (31) constituting a floor surface (33) and a horizontal plane (HP), the floorboard has an edge portion (20) with an edge surface (50) which is located under the horizontal plane **characterized in that** the surface layer (31) is applied on the core to form a floor element (3) in the form of a laminate, said core (30) being made of HDF, the floor element is cut into floor panels (2),
a pressure is applied on the surface of an edge portion (20) of the floor panel such that the core under the surface layer is compressed and the surface layer is permanently bended towards the rear side, whereby
before applying said compression an edge groove (16) is formed at the edge of the floor panel (2), and
after applying said compression a mechanical locking system (9,10, 6,8) is formed at the edge of the floor panel (2).

2. A method as claimed in claim 1, **characterized**
**in that** the surface layer (31) comprises paper sheets impregnated with a thermosetting resin.

3. A method as claimed in claim 1, **characterized**
**in that** the surface layer (31) is a wood veneer.

4. A method as claimed in claim 4, **characterized**
**in that** the edge portion (20) is pressed under heat exceeding 100 degree C.

5. A method as claimed in claim 4, **characterized**
**in that** the edge portion (20) is pressed under heat exceeding 160 degree C.

## Patentansprüche

1. Verfahren zum Herstellen einer Bodenplatte mit einem Verriegelungssystem, einem Kern (30) auf Holzfaserbasis und einer Oberflächenschicht (31), die an der Oberseite des Kerns angeordnet ist, wobei die äußeren flachen Teile der Oberflächenschicht
(31) eine Bodenfläche (33) sowie eine horizontale Ebene (HP) bilden, und die Bodenplatte einen Kantenabschnitt (20) mit einer Kantenfläche (50) aufweist, die sich unter der horizontalen Ebene befindet, **dadurch gekennzeichnet, dass**
die Oberflächenschicht (31) auf den Kern aufgebracht wird, um ein Bodenelement (3) in Form eines Laminats auszubilden, wobei der Kern (30) aus HDF besteht,
das Bodenelement in Bodenplatten (2) geschnitten wird,
ein Druck auf die Oberfläche eines Kantenabschnitts (20) der Bodenplatte so ausgeübt wird, dass der Kern unter der Oberflächenschicht zusammengedrückt wird und die Oberflächenschicht permanent auf die Rückseite zu gebogen wird, wobei
bevor das Zusammendrücken ausgeführt wird, eine Kantennut (16) an der Kante der Bodenplatte (2) ausgebildet wird, und
nachdem das Zusammendrücken ausgeführt ist, ein mechanisches Verriegelungssystem (9, 10, 6, 8) an der Kante der Bodenplatte (2) ausgebildet wird.

2. Verfahren nach Anspruch 1, **dadurch gekennzeichnet, dass** die Oberflächenschicht (31) Papierblätter umfasst, die mit einem wärmehärtenden Harz imprägniert sind.

3. Verfahren nach Anspruch 1, **dadurch gekennzeichnet, dass** die Oberflächenschicht (31) ein Holzfurnier ist.

4. Verfahren nach Anspruch 4, **dadurch gekennzeichnet, dass** der Kantenabschnitt (20) unter Wärme gepresst wird, die 100 °C übersteigt.

5. Verfahren nach Anspruch 4, **dadurch gekennzeichnet, dass** der Kantenabschnitt (20) unter Wärme gepresst wird, die 160 °C übersteigt.

## Revendications

1. Procédé pour fabriquer un plancher, avec un système de verrouillage, une âme à base de fibres de bois (30) et une couche de surface (31) agencée sur la face supérieure de l'âme, les parties plates externes de la couche de surface (31) constituant une surface de plancher (33) et un plan horizontal (HP), le plancher a une partie de bord (20) avec une surface de bord (50) qui est située sous le plan horizontal **caractérisé en ce que**
la couche de surface (31) est appliquée sur l'âme pour former un élément de plancher (3) sous la forme d'un stratifié, ladite âme (30) étant constituée de HDF,
l'élément de plancher est découpé en panneaux de plancher (2),
une pression est appliquée sur la surface d'une partie de bord (20) du panneau de plancher de sorte que l'âme sous la couche de surface soit comprimée et la couche de surface est fléchie de manière permanente vers le côté arrière, de telle manière que
avant l'application de ladite compression une nervure de bord (16) est formée au bord du panneau de plancher (2), et
après l'application de ladite compression un système de verrouillage mécanique (9, 10, 6, 8) est formé au bord du panneau de plancher (2).

2. Procédé selon la revendication 1, **caractérisé en ce que** la couche de surface (31) comprend des feuilles de papier imprégnées avec une résine thermodurcissable.

3. Procédé selon la revendication 1, **caractérisé en ce que** la couche de surface (31) est une feuille mince de bois.

4. Procédé selon la revendication 4, **caractérisé en ce que** la partie de bord (20) est pressée sous chauffage au-dessus de 100 °C.

5. Procédé selon la revendication 4, **caractérisé en ce que** la partie de bord (20) est pressée sous chauffage au-dessus de 160 °C.
